

Jan. 27, 1953

L. J. WEBSTER

2,626,867

LIGHT-SENSITIVE PHOTOGRAPHIC ELEMENT

Filed Dec. 4, 1947

*Fig. 1.*



*Fig. 2*



INVENTOR

LAWRENCE J. WEBSTER

BY *Lynn Barrett Morris*

ATTORNEY

## UNITED STATES PATENT OFFICE

2,626,867

## LIGHT-SENSITIVE PHOTOGRAPHIC ELEMENT

Lawrence J. Webster, Rochester, N. Y., assignor to  
 E. I. du Pont de Nemours & Company, Wilmington, Del., a corporation of Delaware

Application December 4, 1947, Serial No. 789,769

5 Claims. (Cl. 95—7)

1

This invention relates to photographic elements which have a delustered or matte surface. More particularly it relates to photographic elements which have a water-permeable outer layer or strata which has a matte surface.

An object of this invention is to provide photographic elements which have an improved smooth matte surface. A further object is to provide such elements wherein the matting agents are not subject to chemical decomposition by fungi or bacteria. A still further object is to provide such elements in which the matting agents are not readily deformable and are stable over a wide range of temperature conditions. Another object is to provide such elements in a simple and economical manner. Still other objects will be apparent from the following description.

The above objects are attained by the novel photographic elements of this invention which consist of a support, e. g., a film or paper bearing at least one water-permeable silver halide emulsion layer having an outer surface thereof provided with a matte surface by means of finely divided particles of a highly porous siliceous material taken from the group consisting of porous silicon dioxide and porous magnesium silicate.

The highly porous siliceous materials just described should have a particle size so that they fall within the range of 2 to 10 microns in their greatest axial dimension and a dry bulk density of from 2 to 13 pounds per cubic foot of such fine particles. They also possess a specific gravity of about 2.0 to 2.32 and a refractive index of 1.40 to 1.45. They may be disposed throughout the colloid silver halide emulsion layer or they may be uniformly distributed throughout a thin colloid layer which is in intimate contact with the emulsion layer but are preferably distributed in the silver halide layer.

The finely divided particles of the highly porous siliceous materials may be dispersed either in the colloid silver halide coating solution or they may be dispersed in an aqueous solution or dispersion of the colloid binding agent or medium which is mixed with a colloid silver halide emulsion prior to coating the latter to form a light sensitive layer. Uniform dispersion of the novel matting agents described above may be accomplished by passing a mixture of the agent and the binding agent and also the silver halides if desired through a colloid dispersion mill or homogenizer. The aqueous colloid containing the matting agents must be maintained at a temperature above the congealing point of the colloid during the dispersion operation. Similarly when the dis-

2

persion is made in the colloid free from silver halides it should be brought to a temperature above the congealing point before it is added to a silver halide emulsion.

5 Representative photographic papers of this invention are shown in the accompanying drawing which forms a part of this specification. Referring now to the drawing:

Fig. 1 is a schematical cross-section of the photographic paper described in Example II, and

10 Fig. 2 is a schematical cross-section of the photographic paper of Example IV.

The invention will be further illustrated but is not intended to be limited by the following examples.

## Example I

A gelatin solution to be used for the dispersion of a highly porous magnesium silicate was prepared in the following manner:

20 Six grams of photographic gelatin were suspended in 200 cubic centimeters of distilled water at about 75° F. and agitated occasionally. After a soaking period of one hour, the temperature was raised to 120° F. for thirty minutes. The gelatin dissolved completely.

25 Forty grams of porous magnesium silicate (trade name—Magnesol) having a particle size within the 2 to 10 microns range, a specific gravity of 2.0 to 2.35, a refractive index of 1.40 to 1.45 and a dry bulk density of 8 to 12 pounds per cubic foot were stirred into the warm gelatin solution and the mixture was dispersed in a colloid dispersion mill set at a 0.002 inch rotor-stator clearance and operating at a speed of 17,000

30 R. P. M. In passing through the colloid mill all clumps or aggregates of porous magnesium silicate particles existing in the gelatin solution were dispersed so that each individual porous magnesium silicate particle of the basic 2 to 10 micron size was completely wetted by the gelatin suspending solution. Further, after passage through the colloid mill the porous magnesium silicate particles not only were uniformly dispersed in the gelatin solution but exhibited no tendency to reform aggregates or clumps of particles.

## Example II

35 Twenty cubic centimeters of the magnesium silicate-gelatin matte suspension from Example I were added to 250 cubic centimeters of molten gelatin silver chlorobromide emulsion and the latter was coated upon a baryta coated photographic paper and dried. The emulsion surface of the coated paper was uniformly and completely

## 3

delustered to a degree designated by the photographic paper industry as "full-matte." The photographic paper of this example as stated above is illustrated in Fig. 1 of the drawing. Referring now to this figure, a paper support 1 has deposited thereon a baryta coating 2 which in turn carries a gelatin silver chlorobromide emulsion layer 3 which has intimately dispersed therethrough finely divided porous magnesium silicate particles.

## Example III

A porous magnesium silicate-gelatin matte suspension was prepared by the same technique as employed in Example I. Six hundred grams of porous magnesium silicate having the characteristics given in Example I were dispersed in a gelatin solution composed of 90 grams of photographic gelatin dissolved in 3000 cubic centimeters of distilled water. A portion of the resulting dispersion was added to molten gelatin silver chlorobromide photographic emulsion in the proportion of 26 cubic centimeters of the dispersion for each liter of photographic emulsion. Fifteen hundred lineal feet of photographic paper base were coated with this delustered emulsion using production scale coating equipment. No sediment of magnesium silicate formed either in the coating pan or the emulsion receptacles used to continuously replenish the emulsion supply in the coating pan. The photographic paper coating was partially delustered to a degree termed "semi-matte" by the photographic paper industry.

## Example IV

A stock suspension of matting agent was prepared by stirring 150 grams of finely divided porous silicon dioxide, containing a few large aggregates of particles, into 1000 cubic centimeters of 3% aqueous photographic gelatine solution. The suspension was ballmilled for a period of 4 hours until the particle size was from 2 to 10 microns.

Fifteen cubic centimeters of this stock matte suspension were added to 250 cubic centimeters of molten gelatin silver chlorobromide photographic emulsion which was subsequently coated upon a photographic paper base and dried. The resulting product was uniformly delustered. The surface of the emulsion was smooth to the touch, having no rough irregular projections. The smoothness and character of the delustered surface is equal or superior to other commercial delusterants in all respects. The photographic paper of this example, as stated above, is illustrated in Fig. 2 of the drawing. Referring now to this figure, photographic paper base 4 carries a layer 5 of a gelatin silver chlorobromide emulsion which has intimately dispersed therethrough finely divided porous silicon dioxide particles.

## Example V

One hundred and twenty grams of very porous silicon dioxide powder having an apparent dry density of 6.0 pounds per cubic foot were dispersed in an aqueous gelatin anti-abrasion layer formula by passing the mixture through a colloid mill. The particles had a size between 2 and 10 microns. The composition was then coated over a 1500 foot coating of chilled congealed gelatin silver chlorobromide emulsion layer on photographic paper base to form a thin anti-abrasion coating. The double layer unit was then dried. Only very slight delusterant sediment formed in

## 4

the coating pan and emulsion reservoirs during the coating period. The clarity and range of developed silver density on the resulting photographic paper was not impaired by the overlying delusterant or matte layer.

Various colloids can be used in place of gelatin as the binding agents for the silver halide grains and the novel matte-producing agents of this invention. Among such binding agents are albumin, agar-agar, hydrophilic acetals of polyvinyl alcohol and its lower alkyl ethers and esters, hydrophilic cellulose derivatives, e. g., cellulose acetate; etc.

The amount of the matte-producing agents may vary depending upon the particular colloid binding agent and the effect desired. In general from 0.005 to 0.6 parts of the porous siliceous particles should be used per part of colloid binding agent.

20 The porous silicon dioxides and magnesium silicates when used in accordance with this invention result in products which have numerous advantages. The particles are white in appearance and have a density very close to that of fluid gelatin and hence do not tend to settle but on the contrary form stable suspensions or dispersions in colloid solutions. They do not separate out in the coated layers and thus the layers have good uniformity, especially near the surface.

30 A further advantage of the use of the porous silicon dioxides and magnesium silicates is that much less milling time is necessary to reduce the particle size of outsize particles to the desired limits and to break up any aggregates. The 35 highly porous siliceous materials just described result in a greater degree of transparency of the delusterant so that the photographic likeness of an object can be reproduced on the photographic paper with greater clarity and with a greater range of reduced silver density. They may be 40 successfully used in thin anti-abrasion layers without any subsequent opaquing or graying effect on the gelatin silver halide under-layer. Dense silica particles do not produce similar results.

45 As many widely different embodiments of this invention can be made without departing from the spirit and scope thereof, it is to be understood that the invention is not to be limited except as defined by the claims.

50 What is claimed is:

1. A photographic element comprising a support bearing a gelatino silver halide emulsion layer containing finely divided particles of porous magnesium silicate having a particle size of 2 to 10 microns, a dry bulk density of 2 to 13 pounds per cubic foot and a specific gravity of 2.00 to 2.35, said particles being present in an amount of 0.005 to 0.6 part per part of gelatin by weight.

55 2. A photograph element comprising a paper support bearing a gelatino silver halide layer containing finely divided particles of a highly porous magnesium silicate having a particle size of 2 to 10 microns, a dry bulk density of 2 to 13 pounds per cubic foot and a specific gravity of 2.00 to 2.35, said particles being present in an amount of 0.005 to 0.6 part per part of gelatin by weight.

60 3. A photographic element comprising a paper support bearing a water-permeable silver halide emulsion layer on which is deposited a thin water-permeable colloid layer containing finely divided particles of a highly porous magnesium silicate having a particle size of 2 to 10 microns, a dry bulk density of 2 to 13 pounds per cubic foot and a specific gravity of 2.00 to 2.35, said particles

being present in an amount of 0.005 to 0.6 part per part of colloid by weight.

4. A photographic element comprising a paper support bearing a gelatin silver halide emulsion layer on which is deposited a thin gelatin colloid layer containing finely divided particles of a highly porous magnesium silicate having a particle size of 2 to 10 microns, a dry bulk density of 2 to 13 pounds per cubic foot and a specific gravity of 2.00 to 2.35, said particles being present in an amount of 0.005 to 0.6 part per part of gelatin by weight.

5. A photographic element comprising a flexible sheet support and at least one gelatin-containing layer on the support, said element having light-sensitive silver halide grains dispersed in the gelatin binding agent and finely divided particles of porous magnesium silicate having a particle size from 2 to 10 microns, a dry bulk density of 2 to 13 pounds per cubic foot and a specific gravity of 2.00 to 2.35 dispersed in the gelatin binding

5

agent, said particles being present in an amount of 0.005 to 0.6 parts per part of gelatin and in intimate association with the silver halide grains and in the outer stratum of gelatin.

LAWRENCE J. WEBSTER.

## REFERENCES CITED

The following references are of record in the file of this patent:

## UNITED STATES PATENTS

| Number    | Name          | Date          |
|-----------|---------------|---------------|
| 1,989,879 | Murck         | Feb. 5, 1935  |
| 2,322,037 | Lindquist     | June 15, 1943 |
| 2,384,093 | Holmen et al. | Sept. 4, 1945 |
| 2,433,515 | Jahoda        | Dec. 30, 1947 |

## FOREIGN PATENTS

| Number | Country       | Date |
|--------|---------------|------|
| 3,736  | Great Britain | 1900 |